

## UNITED STATES PATENT OFFICE

2,018,588

PROCESS OF FILLING LEATHER AND THE  
RESULTING PRODUCTLester M. Whitmore, Salem, Va., assignor to Leas  
and McVitty, Inc., Philadelphia, Pa., a corpo-  
ration of DelawareNo Drawing. Application July 27, 1934.  
Serial No. 737,290

14 Claims. (Cl. 149—4)

My invention relates to an improved leather product and to the process of making it, and more particularly it relates to an improved leather product, especially applicable as a heavy sole leather.

One object of my invention is to provide a leather product of increased solidity, and increased thickness and weight, which properties are obtained in the leather without the necessity 10 of loading the product with a water-soluble filler as has previously been the case.

A further object of my invention is to furnish to the trade a leather, particularly adapted for use as sole leather, which possesses high wear-resistant qualities and high resistance to water penetration and to the softening effects normally encountered in the presence of moisture or high humidities.

Still another object of my invention is to provide a leather with a marked decrease in the tendency of the product to air-burn during the drying operation and for the tanning extracts to bleed to surface during drying or when the product is worked in a damp condition.

These and other objects including the provision of a novel process of preparing the leather product will be apparent hereinafter from a consideration of the specification and claims.

Heretofore in the tanning of leather with the natural vegetable tanning extracts, particularly those containing catechol tanning materials, difficulties have been encountered in the process, and in the manufacture of heavy leathers, particularly sole leather, various water soluble materials as fillers have been added to the leather during the process in an attempt to increase the solidity, thickness, weight, and resistance to wear and water penetration. Due to the solubility of the vegetable tanning agents in water and of the water soluble fillers, these materials during manufacture tend to bleed to the surface, particularly during drying or when the leather is worked in a damp condition. Additionally, the leather tends to air-burn during the drying resulting in an inferior product. Furthermore, the finished product, due to the presence of water-soluble material therein, is not characterized by high resistance to wear or water penetration since in the presence of moisture or high humidities, 50 a dissolving action on the water-soluble material takes place.

The process of the present invention overcomes or reduces to a minimum all of the disadvantages of the previous processes, and the product possesses properties which have previously been

sought but have only been obtained to a small degree.

In the process of the present invention, the active tanning agents of the extracts are converted chemically into insoluble products which are then retained permanently between and on the fibres and fibrils of the leather. The chemical conversion of the tanning agents into insoluble material is brought about by a reaction between them, an aldehyde and an ammonium salt. Since the active tanning agent after performing its tanning function is rendered insoluble, there is no tendency for the leather to bleed or to air-burn. Furthermore, the finished product, due to the presence of the insoluble material 15 therein, possesses increased weight, thickness, solidity, and resistance to wear. The product also offers a higher resistance to water penetration and to softening in the presence of moisture or high humidities. The reaction of the tanning 20 agents with the aldehyde and the ammonium salt also gives an antiseptic effect to the leather which reduces the growth of molds normally encountered with damp leather. By the process of the present invention, a leather is easily obtained 25 having a degree of tannage of 110° to 140° or even higher based on the relation between combined tannin and hide substance as determined by the official method of the American Leather Chemists Association, which will be recognized 30 as higher than that previously encountered in such products.

The process of the present invention may be carried out with any type of hide and any of the usual vegetable tanning extracts, particularly 35 those containing catechol tannins, may be used as the tanning material. For example, the following materials or extracts have been found to be applicable for use:—mangrove, wattle, quebracho 3% bisulphited, quebracho 6% bisulphited; gam- 40 bier, hemlock, cutch, chestnut, chestnut oak, myrabolans, valonia, divi-divi, and the like. The aldehyde which is employed preferably is formaldehyde due to its availability and cheapness but other aldehydes including acetaldehyde, fur- 45 furaldehyde, and benzaldehyde may be used. Any salt containing the ammonium radical will satisfactorily react, for example, ammonium sulphate, ammonium chloride, ammonium oxalate, or ammonium phosphate. 50

The reaction of the aldehyde and the ammonium salt with the tanning agents to deposit insoluble material between and on the fibers and fibrils of the leather is not strictly speaking a tanning process but rather a filling or finishing

process since the hide is tanned as previously with the tanning agent. The amount of tanning agent employed and the steps of the tanning process may be the same as has previously been the practice with the particular type of hide to be tanned and the particular type of leather to be manufactured. The order of addition of the materials is immaterial but it is desirable that the treatment with the aldehyde shall take place after the leather has been tanned, at least to some extent, and the process is particularly applicable for the treatment of tanned leather. The three reactants may be added simultaneously but preferably the aldehyde is not added until the tanning extracts have been absorbed by the hide or leather. The ammonium salt may be added with the tanning agent, simultaneously with the aldehyde, or thereafter. The aldehyde and/or ammonium salt may be reacted with the tanning extract in the wheel, drum, temper bath, dry dip, or elsewhere in the process.

25 The amounts of tanning extract, aldehyde, and ammonium salt employed are not critical and depend upon the degree of improvement desired. In general, it has been found advisable to use at least 3% to 4% of aldehyde, and about 5% of the ammonium salt on the basis of dry extract to obtain the optimum results, but additional amounts of these materials are not detrimental to the leather. As examples, the following proportions have been found to give satisfactory results: 30 50 cubic centimeters of 40° Twaddell clarified quebracho extract, 1 gram of ammonium chloride, and 4 cubic centimeters of commercial 40% formaldehyde solution; or 50 cubic centimeters of 40° Twaddell clarified quebracho extract, .5 grams of ammonium chloride, and 5 cubic centimeters of commercial 40% formaldehyde solution.

35 The following specific examples are given merely by way of illustration, and it will be obvious that many variations may be made therein without departing from the essential features of the invention.

#### Example I

40 Leather is drummed in the usual manner with quebracho extract to which has been added 5% of ammonium sulphate on the dry basis. The stock is piled down over night to absorb the load and bleached to clear the surface of the leather. It is then dipped fifteen minutes in a solution of 45 formaldehyde containing 20% of this ingredient, piled over night to react and fix, and then oiled off and finished in the usual manner.

#### Example II

50 Rough dry leather which has had one wheel load is dry dipped in a 75 Barkometer dry dip consisting of 95 parts of clarified quebracho and 5 parts of ammonium sulphate on a dry basis. Coming from the dry dip, the leather is dipped 55 fifteen minutes in a solution of 20% formaldehyde and is then given an oil wheel load of Epsom salts, sugar, and oil, set out, and finished in accordance with the usual practice.

#### Example III

60 Leather from the yard may be drummed with 20% of its weight of 40 Twaddell clarified quebracho extract plus desired amounts of sugar and oil, and .5% of its weight of ammonium chloride on the dry basis. When dry, the leather is 65 dipped in a 4% formaldehyde solution for ten minutes, piled down for twenty-four hours to set, and redried. The leather may then be dry

dipped if desired in the usual manner to give additional water soluble load, after which it is finished as usual.

65 In some instances, it will be found desirable to react the formaldehyde remaining in contact with the leather after the completion of the reaction with a compound capable of converting it into another substance in order to avoid the presence of formaldehyde fumes in subsequent operations. This may be accomplished by bringing a compound capable of reacting with formaldehyde into contact with the leather after the precipitation of the insoluble compound as herein described and as typical of these substitutes, a bisulphite compound or an ammonia derivative such as urea may 15 be mentioned.

I claim:

1. The process of filling leather which comprises reacting a vegetable tanning extract, aldehyde, and an ammonium salt together between 20 and on the fibres and fibrils of leather to deposit an insoluble material therebetween and thereon.

2. The process of filling leather which comprises reacting a vegetable tanning extract containing a catechol tannin, formaldehyde, and 25 an ammonium salt together between and on the fibres and fibrils of leather to deposit an insoluble material therebetween and thereon.

3. The process of filling leather which comprises reacting a vegetable tanning extract containing a catechol tannin, formaldehyde, and ammonium sulphate together between and on the fibres and fibrils of leather to deposit an insoluble material therebetween and thereon.

35 4. The process of filling leather which comprises reacting a vegetable tanning extract, aldehyde, and an ammonium salt together between and on the fibres and fibrils of leather to deposit an insoluble material therebetween and thereon, the aldehyde being present in the neighborhood of 3% to 4% and the ammonium salt being present in the neighborhood of 5% figured as ammonium sulphate and based on the dry extract.

45 5. The process of filling leather which comprises reacting a vegetable tanning extract containing a catechol tannin, formaldehyde, and an ammonium salt together between and on the fibres and fibrils of leather to deposit an insoluble material therebetween and thereon, the 50 formaldehyde being present in the neighborhood of 3% to 4% and the ammonium salt being present in the neighborhood of 5% figured as ammonium sulphate and based on the dry extract.

55 6. The process of filling leather which comprises reacting a vegetable tanning extract containing a catechol tannin, formaldehyde, and ammonium sulphate together between and on the fibres and fibrils of leather to deposit an insoluble material therebetween and thereon, the 60 aldehyde being present in the neighborhood of 3% to 4% and the ammonium sulphate being present in the neighborhood of 5% based on the dry extract.

65 7. The process of filling leather which comprises absorbing a vegetable tanning extract between and on the fibres and fibrils of leather, and thereafter reacting an aldehyde and an ammonium salt therewith to deposit an insoluble material between and on said fibres and fibrils.

70 8. The process of filling leather which comprises absorbing a vegetable tanning extract containing a catechol tannin between and on the fibres and fibrils of leather, and thereafter reacting formaldehyde and an ammonium salt there-

with to deposit an insoluble material between and on said fibres and fibrils.

9. Filled leather containing the insoluble reaction product of a vegetable tannin extract, an aldehyde, and an ammonium salt between and on the fibres and fibrils thereof.

10. Filled leather containing the insoluble reaction product of a vegetable tannin extract containing a catechol tannin, formaldehyde, and an ammonium salt between and on the fibres and fibrils thereof.

11. Filled leather containing the insoluble reaction product of a vegetable tannin extract containing a catechol tannin, formaldehyde, and ammonium sulphate between and on the fibres and fibrils thereof.

12. Filled leather having a degree of tannage of at least 110° determined by the official method of the American Leather Chemists Association.

and containing the insoluble reaction product of a vegetable tannin extract, an aldehyde, and an ammonium salt between and on the fibres and fibrils thereof.

13. Filled leather having a degree of tannage of at least 110° determined by the official method of the American Leather Chemists Association, and containing the insoluble reaction product of a vegetable tannin extract containing a catechol tannin, formaldehyde, and an ammonium salt between and on the fibres and fibrils thereof.

14. Filled leather having a degree of tannage of at least 110° determined by the official method of the American Leather Chemists Association, and containing the insoluble reaction product of a vegetable tannin extract containing a catechol tannin, formaldehyde, and ammonium sulphate between and on the fibres and fibrils thereof.

LESTER M. WHITMORE.